

## UNITED STATES PATENT OFFICE.

THEODORE H. BROWN, OF MINNEAPOLIS, MINNESOTA, ASSIGNOR OF SEVEN TWENTY-FOURTHS TO J. C. DONAHUE AND SEVEN TWENTY-FOURTHS TO DAVE BLISS, BOTH OF MINNEAPOLIS, MINNESOTA.

## COMPOSITION FOR MAKING SHINGLES.

1,263,847.

Specification of Letters Patent. Patented Apr. 23, 1918.

No Drawing.

Application filed August 27, 1917. Serial No. 188,523.

To all whom it may concern:

Be it known that I, THEODORE H. BROWN, a citizen of the United States, and a resident of Minneapolis, in the county of Hennepin and State of Minnesota, have invented certain new and useful Improvements in a Composition for Making Shingles, of which the following is a specification.

One object of my invention is to provide an improved composition for making shingles and an improved and inexpensive shingle produced from the compound.

Another object of my invention is to provide in a compound and shingles produced therefrom, means for strengthening the resultant shingle.

With these and incidental objects in view the invention consists of certain products formed in a composition as described in the following specification.

I prefer to form my compound of one-eighth of a bitumen and seven-eighths of coal dust.

I prefer to use as a bitumen the asphaltum product produced from the Texas fields, and ordinarily known as the Texas asphaltum, and as a coal dust I prefer to use what is called slack dust.

To combine the two products the coal dust must first be heated to a partial incandescence, the bitumen then mixed with the heated coal, and the compound agitated by any suitable means to thoroughly mix the two products.

When the products have been thoroughly mixed they are then pressed together, either under a flat pressure device or under rollers, and the heavier the pressure the better the product all things being equal.

After the product has come from the rolls I then prefer to coat one or both sides of the resultant sheet with common salt, NaCl, by

sprinkling the salt on the surface of the sheet and the heat of the compound melts the salt, chemically mixes the products, and gives a fire retardant sheet.

To give additional stiffness to the sheet so formed, I sometimes press the compound between two sheets of gauze, the pressure incorporating the gauze within the body of the sheet so that there is a certain amount of compound outside of the two sheets so incorporated, and this use of gauze may be employed either with or without the coat of salt.

While I have described my invention in one particular manner and as a combination of certain products, I do not wish it to be understood that I limit myself to this way, as it is evident the invention may be varied in many ways within the scope of the following claims.

## Claims:

1. A compound for making roofing shingles formed of seven-eighths slack coal dust heated to partial incandescence and then mixed with one-eighth of bitumen thoroughly mixed with the coal dust in its partial incandescent state and the compound thoroughly amalgamated through pressure.

2. A compound for making roofing shingles formed by heating coal dust to a partial incandescence, mixing with the coal dust, while it is so heated, one-seventh of the same weight of a bitumen, and agitating the mixture so formed and pressing the mixture into a sheet.

3. A compound for making shingles and the like comprised of bitumen and coal dust thoroughly mixed, the coal dust being partially oxidized before the bitumen is combined therewith.

THEODORE H. BROWN.